# EUROPEAN PATENT SPECIFICATION

(11) **EP 1 569 777 B1**
(45) Date of publication and mention of the grant of the patent: **04.04.2007**
(21) Application number: 03778360.2
(22) Date of filing: 08.12.2003
(51) Int. Cl.: B28B 7/36

(54) **A METHOD FOR CREATING A NON-POROUS FAIR-FACE SURFACE WHEN CASTING CONCRETE**
VERFAHREN ZURERZEUGUNG EINER NICHTPORÖSEN GLATTPUTZFLÄCHE BEI GIESSEN VON BETON
PROCEDE D'OBTENTION D'UNE SURFACE EN BETON DE PAREMENT NON POREUSE LORS DU COULAGE DU BETON

(30) Priority: 10.12.2002 FI 20022173
(43) Date of publication of application: 07.09.2005
(73) Proprietor: Naamanka, Janne Samuli, 02770 Espoo (FI)
(72) Inventor: Naamanka, Janne Samuli, 02770 Espoo (FI)
(74) Representative: Laitinen, Pauli Sakari
(86) International application number: PCT/FI2003/000936
(87) International publication number: WO 2004/052604

(56) References cited:
- EP-A2- 0 375 924
- FR-A- 2 071 454
- GB-A- 1 127 296
- US-A- 4 112 173
- DATABASE WPI Week 198119, Derwent Publications Ltd., London, GB; Class A93, AN 1981-33496D, XP002990417 & JP 56 028 971 A (KOYO SANGYO CO LTD) 23 March 1981
- PATENT ABSTRACTS OF JAPAN vol. 2003, no. 12 05 December 2003 & JP 2003 268924 A (NISSHOKU CORP) 25 September 2003
- DATABASE WPI Week 199950, Derwent Publications Ltd., London, GB; Class A93, AN 1999-584745, XP002229181 & JP 11 254 416 A (ASAHI KASEI KOGYO KK ET AL) 21 September 1999

## Description

The present invention relates to a method for creating a non-porous surface when casting concrete.

Concrete being cast copies onto its surface a negative image of the surface structure of the formwork material. In old structures, the pattern of rough-sawn planks used in plank formwork is often visible. Plank formwork has the advantage that the planks absorb water from the surface of the freshly cast concrete and thus blisters are seldom seen on surfaces cast in this way. However, the formwork material must always be treated with so-called formwork stripping agent, which ensures that the formwork will detach from the hardened concrete in one piece, without breaking the new concrete surface. Treatment with stripping agent decisively reduces the planks' water absorption. In present-day concrete technology, the use of plank formwork has diminished considerably. Thus, at present, materials that do not absorb water are used, for example, treated plywood and steel.

The quality of the new concrete surfaces has not come up to expectations, but often leaves much to be desired. Quality requirements have therefore been issued for surfaces, depending on the surface treatment to be given afterwards to the concrete surface, and on the distance from which the concrete surface will be seen. According to the present guidelines issued by the Finnish Concrete Association (Concrete Surfaces, by 40), in the highest quality grade, 20 pores per square metre are permitted on the surface of concrete cast against horizontal formwork. Double this number of pores are allowed in a surface cast against vertical formwork. Keeping the numbers of pores beneath the guidelines generally demands the use of varnished timber formwork. Even then, it is often doubtful whether the surface created will meet the above requirements. It is therefore increasingly uncommon to see surfaces cast against untreated formwork.

Very often, it is imagined that the pores arising in a concrete surface come from the collection, in the interface between the formwork and the concrete, of the air that is naturally trapped in the concrete. However, the pores usually come from the separation of water contained in the concrete mass, as the concrete compacts.

The high surface tension of water causes a large angle of contact between a drop of water and the formwork material, which causes the water to separate into large drops against the concrete and thus form a blister in the hardening concrete. In practice, fresh concrete must be compacted by vibration, and this is the force that collects the water as drops on the formwork surface.

In Japanese publication 56028971 a plastic film is glued on a plywood plate and the manufactured combination is used as a material for a concrete casting form. In this publication the corona treatment is used to facilitate glueing of the plastic film.

In US patent 4112173 electric field is used when paper is covered with molten plastics.

British publication 1127296 describes plastics coated paper, which may be also corona treated, as a form material for gypsum casting.

The present invention is therefore intended to create a method, with the aid of which a fair-face surface, of very even quality and without blisters, can be achieved in concrete.

This is achieved in the manner described as characteristic in the accompanying Claims, whereby the pre-amble of claim 1 is disclosed by JP-A-56028971.

In general, it can be said that the invention is made by using, on the surface of the formwork, a membrane of special material that lies against the concrete being cast, with the aid of which the formation of blisters is prevented.

According to one preferred embodiment, the casting membrane has a three-layer structure, which can comprise a paper-based middle layer and a plastic coating on each side of it. The use of this structure creates a material for the casting membrane that is sufficiently thin and is also sufficiently inelastic and stiff. In the casting membrane, the paper acts precisely as a stiffener and reduces stretch. However, a membrane, with a plastic coating only on the side of the membrane that comes against the concrete being cast, is also practicable.

However, coating the casting membrane with plastic on both sides will naturally act as more effective moisture-proofing than a membrane surfaced on one side, as the water in the damp concrete will not swell the paper mass.

The casting membrane according to the invention is manufactured in a conventional manner by coating at least one side of a cellulose-based paper web with a membrane of a suitable plastic, or of a plastic composition. After this, the membrane is subject to an electrical treatment, which is usually termed corona treatment. Its principle is that, by exploiting electrical discharges, the surface of the plastic coating is broken at the micro-level. Naturally, the corona treatment can be performed on both sides of the membrane, in cases in which both surfaces are coated with plastic, but it is performed at least on the surface that lies against the concrete being cast during casting.

The aforesaid corona treatment has a positive effect on the surface tension of water. This reduction in surface tension creates precisely a fair-face surface on the concrete that is without blisters and is of an even quality. It is assumed that the excellent casting surface arises because the water in the concrete cast against the formwork can flow in the micro-level passages and does not remain as drops between the concrete and the membrane, which would create blisters in the concrete surface.

The above behaviour of a drop is also illustrated in the accompanying drawings, in which Figures 1 a and 1 b show two parallel figures as a series showing the assumed behaviour according to the prior art (Fig. 1 a) and the behaviour when using a membrane according to the invention (Fig. 1 b). The reference number 1 represents the membrane according to the invention while number 2 represents the water drop. The reference number 3, on the other hand, represents the angle of contact between the membrane and the drop, which, in the case of a large drop of water is obtuse, while the angle when using a membrane according to the invention is acute and the drop is widely spread.

The use of the said casting membrane permits the process of casting large units, without creasing or folding. Practical experiments have shown that the method actually works excellently and that with its aid a fair-face surface of excellent quality can be obtained.

A further additional advantage of the invention that can be mentioned is that, when using a casting membrane according to the invention, there is usually no need to use a separate stripping agent, as the formwork material will detach from the hardened concrete easily and completely. In the material according to the invention, there is a stiff non-creasing cellulose-based layer of material, usually of paper, surfaced with a plastic membrane. In a normal situation, the low surface energy of the plastic membrane would, as such, cause the formation of a water drop as described above and through it the formation of a blister in the concrete surface being created. However, as stated above, the surface energy of the plastic membrane can economically and effectively be increased using the said electric discharge treatment, i.e. corona treatment. In corona treatment, the plastic surface is treated using an electric current, which causes sparking and forms ozone. Together, these factors increase the energy of the plastic surface and thus reduce the angle of contact between the formwork surface and the water drop to such an extent that a water drop, and through it a pore, cannot form.

## Claims

1. A method for creating a non-porous, fair-face surface, when casting concrete, in which a casting membrane **characterized in that** said casting membrane (1) is used between the concrete being cast and the formwork, the casting membrane **characterized in that** said casting membrane (1) is formed of a plastic coating, **characterized in that** said casting membrane (1) is treated using an electrical discharge treatment, at least on the surface against the concrete being cast.

2. A method according to Claim 1, **characterized in that** the electrical discharge treatment is a so-called corona treatment.

3. A method according to Claim 1, **characterized in that** a casting membrane is used on the surface of the formwork, which is formed of a cellulose-based layer, on both sides of which is a plastic coating, which is corona treated, at least on the surface lying against the concrete.

## Patentansprüche

1. Verfahren zur Schaffung einer nicht-porösen Sichtbeton-Oberfläche beim Gießen von Beton, worin eine Gussmembran (1) zwischen dem zu gießenden Beton und der Schalung eingesetzt wird, welche Gussmembran aus einem Kunststoffüberzug ausgebildet ist, **dadurch gekennzeichnet, dass** besagte Gussmembran (1), zumindest an der dem zu gießenden Beton zugewandten Oberfläche durch eine elektrische Entladungsbehandlung behandelt ist.

2. Verfahren nach Anspruch 1, **dadurch gekennzeichnet, dass** die elektrische Entladungsbehandlung eine so genannte Koronabehandlung ist.

3. Verfahren nach Anspruch 1, **dadurch gekennzeichnet, dass** auf der Oberfläche der Schalung eine Gussmembran verwendet wird, die aus einer Schicht auf Cellulosebasis gebildet wird, auf deren beiden Seiten ein Kunststoffüberzug ist, der zumindest auf der dem Beton zugewandten Oberfläche Korona-behandelt ist.

## Revendications

1. Méthode pour créer une surface de parement non poreuse, dans laquelle une membrane de coulage (1) est utilisée, lors du coulage du béton, entre le béton à couler et le coffrage, la membrane de coulage étant formée d'un enduit plastique, **caractérisée en ce que** ladite membrane de coulage (1) est traitée en utilisant un traitement à décharge électrique, du moins sur la surface qui se trouve contre le béton à couler.

2. Méthode selon la revendication 1, **caractérisée en ce que** le traitement à décharge électrique est un traitement appelé traitement corona.

3. Méthode selon la revendication 1, **caractérisée en ce que** la membrane de coulage est utilisée sur la surface du coffrage, celle-ci étant constituée d'une couche à base de cellulose, les deux faces de la membrane ayant un enduit plastique traité corona, du moins sur la surface située contre le béton.
